

W. E. NICKERSON.  
PROCESS OF HARDENING STEEL.  
APPLICATION FILED AUG. 12, 1907.

1,129,113.

Patented Feb. 23, 1915.

2 SHEETS—SHEET 1.



Fig. 1.



Fig. 2.



Fig. 3.

Witnesses:  
Harry C. Helbig  
Charles A. Scheuler

Inventor  
William E. Nickerson  
By his Attorney  
Dunn, Tufts & Clarke

W. E. NICKERSON.  
PROCESS OF HARDENING STEEL.  
APPLICATION FILED AUG. 12, 1907.

1,129,113.

Patented Feb. 23, 1915.

2 SHEETS-SHEET 2.



*Fig. 5.*



Witnesses:  
Harry C. Higby  
Charles A. Schenber.

Inventor  
William E. Nickerson  
By his Attorney  
Orin Durbin & Clarke

# UNITED STATES PATENT OFFICE.

WILLIAM E. NICKERSON, OF CAMBRIDGE, MASSACHUSETTS.

## PROCESS OF HARDENING STEEL.

1,129,113.

Specification of Letters Patent. Patented Feb. 23, 1915.

Application filed August 12, 1907. Serial No. 388,078.

To all whom it may concern:

Be it known that I, WILLIAM E. NICKERSON, of the city of Cambridge, county of Middlesex, and Commonwealth of Massachusetts, have invented certain new and useful Improvements in Processes of Hardening Steel for Use in the Manufacture of Cutting Implements or Tools, of which the following is a full, clear, and exact specification.

My invention relates to certain new and useful improvements in methods or processes of treating steel, and more especially to the hardening of steel blanks for use in the manufacture of cutting implements or tools.

As is well known, in order to produce a sharp and durable cutting edge, it is necessary that the material be suitably hardened, and while the hardness of steel will depend, to some extent, upon the constitution or proportions of the ingredients thereof, the hardness of any given piece may be varied within very wide limits by treatment, and especially by heat treatment.

The usual method of hardening steel consists in heating it in a suitable furnace to a desired predetermined temperature, and then suddenly chilling it by plunging in a cold bath of oil or water. Such treatments, however, while satisfactory in handling objects of moderate size, fall far short of the desired efficiency when applied to thin sheets, for instance, blanks five or six one-thousandths of an inch thick, such as are employed in the manufacture of the razor blades described in United States Letters Patent, Number 775,134 issued to King C. Gillette November 15, 1904; and my invention, while adapted for use in the manufacture of many different articles, is particularly useful in hardening such thin steel sheets or blanks, or in cases where the damage to the surface by oxidation or burning caused by the usual methods of hardening would be objectionable.

I have found that to obtain the highest quality and uniformity of product, it is necessary that the heating operation be so performed that the temperature of the whole mass under manipulation be raised uniformly to the desired temperature, and that the chilling thereof be as nearly instantaneous throughout the entire blank as possible. It is also desirable that the heat be applied quickly as well as uniformly, as

a gradual heating is apt to cause a deterioration of the material. Furthermore, steel in a highly heated condition unites very freely with the oxygen of the air and thus more or less surface oxidation takes place, often to the detriment of the finished article.

The burning of the surface or forming of scale by oxidation occurs more or less in all of the processes of hardening heretofore in use, but in view of the size or mass of the articles, the inconsiderable amount thereof has been insufficient to impair seriously the quality of the finished product. In treating thin sheet plates or blanks, however, of the character referred to above, and which are required to be of the highest degree of excellence and uniformity, the defects above referred to are a serious detriment, and my present invention is intended to overcome them, or to reduce them to a minimum. Other difficulties are also met with in the heating and chilling of thin blanks, such as the liability to buckle or become distorted if the heating and chilling are not performed with sufficient uniformity throughout the entire mass, and it is the object of my invention to obviate or reduce to a minimum all these disadvantages, and to produce a finished article of the highest degree of excellence, with the necessary hardness and uniformity, and the method which I have found very satisfactory is as follows: I take thin steel blanks of the desired size and shape, and if the desired article is the razor blade hereinbefore referred to, I take thin sheet steel blanks cut from rolled sheets or ribbons, and preferably subject them to a preliminary heating operation by which their temperature will be quickly raised, so that when the final heating takes place the danger of buckling or distortion will be reduced to a minimum. This preliminary heating is preferably accomplished by subjecting the blanks to heat radiated from a metallic body which has been raised by means of blow pipes or other suitable apparatus to a temperature of, say, three hundred or four hundred degrees Fahrenheit. The blank is subjected to this radiated heat until it is uniformly raised to about the temperature mentioned. Thus the danger of producing strains or of burning out the surface carbon will be reduced to a minimum and the blank raised to the preliminary temperature without injurious effect.

The blanks so treated are then preferably subjected to a further heating which raises the temperature to the desired degree, this depending largely upon the object or use to which the finished article is to be put, and in order to produce a uniform product it is very important that this final heating be accurately timed and regulated. This may be successfully accomplished by subjecting the blanks to a blast flame of constant temperature for a definite period of time; or, as I prefer to do, by placing them between a pair of metallic heating members which are maintained at a constant temperature by means of blow pipes or other suitable apparatus. The heating of the blanks between the hot surfaces not only prevents, to a very large extent, the burning of the surface, but it prevents strain and the distortion of the blanks and keeps them in desired shape and condition. In addition to this, if the heating bodies be of considerable size or mass, the temperature of the blanks can be successfully determined and maintained with great accuracy and uniformity, while at the same time the heated blanks are protected against oxidation, such as would occur were they maintained freely accessible to the open air.

After the blanks have been raised to the desired temperature, they must be rapidly cooled, and this operation is generally known as quenching. The greater the rapidity of this quenching operation, the more perfect will be the finished article, and I have found that a very successful method is to place the heated blanks between cold surfaces, such as metallic bodies of relatively large mass, which may be kept cool by means of a water circulation or other device, and this will be found to produce a most efficient article. I also find it desirable, in some cases, to employ considerable pressure in the quenching operation, as by this means any distortions or strains are removed, and the finished article is uniformly cooled and retained in the desired shape. I have also found it desirable to subject the hot blanks to the action of a hammer blow for the purpose of insuring their being in the desired condition when the final chilling takes place, and in practice I have found it most desirable to perform this last mentioned operation by transferring the blank, in its heated condition, to a cold, flat surface and then striking it with a similar cold surface, which latter is pressed firmly upon the blank after striking the blow and remains in place until the blank is thoroughly cooled.

In carrying out either the heating or chilling operations above described, it is especially desirable that the metal blocks upon or between which the blanks are treated be relatively of large size or mass compared with the blank, so that the change in tem-

perature thereof by reason of contact with the blank will be extremely small. When properly proportioned, blanks can be properly hardened with great rapidity and can thus be produced in large quantities of a very uniform character. The employment of the preliminary heating operation will be found valuable in carrying out my process, for the reason that it permits of the delivery to the heating blocks of the blanks at such a temperature as to render them less liable to produce any change in the condition of said blocks.

In the accompanying drawing forming part of this application, I have shown types of apparatus which will be found useful in carrying out the foregoing method.

In these drawings, Figure 1 illustrates a device designed to be used in performing the first heating operation. Fig. 2, an apparatus designed to perform the second or final heating operation. Fig. 3 shows one of the parts illustrated in Fig. 2. Fig. 4 discloses an apparatus for chilling or chilling the blank when heated, and Fig. 5 is a horizontal section through one of the chilling members in Fig. 4.

Referring to Fig. 1, the reference numeral 1 indicates the blank held by the carrier 2. Any suitable means may be employed for holding the blank on the carrier but I prefer to use suction means such as are well known in the art and which need not be here described. The heating block or conductor 3 is maintained at the desired temperature by means of blow pipes 4, 4, 4, suitably arranged and regulated, and the blank to be heated is brought within the heat zone above the heating block 3, and is held there for a sufficient time to raise it to the desired temperature. The use of the radiated heat from a heated metallic body is extremely effective for the reason that the blank is not subjected to the direct action of the burning gases of the flames which would tend to injure it, and at the same time the temperature can be more easily regulated than when a direct flame is employed.

In Fig. 2, two heating blocks or conductors 5, 6, are shown, between which the blank, which has received the preliminary heating, is placed. These blocks are subjected to the constant action of blowpipes or blasts 4, 4, 4, 4, 4, and, being of considerable size, are thus maintained at a uniform temperature. When a blank is placed upon the lower block, the upper one is then pressed down thereon and the heat of the blocks is thus transmitted to the blank by conduction and also by reason of the blanks being completely buried in the heat zone. It may be desirable to groove or corrugate the contacting surfaces of the blocks as shown at 7 in Fig. 3, for by so doing, any sticking of the blank to the block will be prevented. A

blank treated as thus described will be gradually raised to the desired temperature without strain or distortion and is then ready for the chilling operation which I prefer to carry out by means of the apparatus shown in Figs. 4 and 5. This consists of a pair of chilling blocks 8, 9, which may be hinged together as shown. These blocks have recesses 10 therein with inlet and outlet pipes 11, 12, through which a constant stream of water is caused to pass for the purpose of maintaining the blocks at a comparatively low temperature. The blocks are caused to approach one another with a rapid motion or blow and are adapted to be held together firmly after the blow by means of the pivoted arm 13 carrying the roller 14 which bears upon the upper surface of block 9, the lever being operated by a weight 15 connected by a cord 16 thereto. In using this apparatus the blank after having received its final heating in the apparatus disclosed in Fig. 2, is immediately transferred to the lower block 9 as shown. The upper block then drops, striking the blank which is then clamped firmly between the two. The chilling is thus produced by conduction from the cold blocks, and takes place evenly throughout the entire blank, which at the same time, is held flat and any distortion or strain prevented.

It is important in both heating and chilling operations that the heating or chilling blocks be comparatively large in size or mass with respect to the blank operated upon. By this means the temperature of the blocks will be practically unaffected by contact with the blank and will remain comparatively uniform when treating a large number of blanks. This is extremely important when a great number of articles must be turned out with the necessary rapidity and uniformity.

It is obvious that in practising my invention, several of the steps described may be omitted or not, without departing from the spirit of the invention, and I do not wish to be understood as limiting myself to a process which includes all of the steps heretofore described, but what I claim and desire to secure by Letters Patent is:

1. The method of hardening thin steel blanks, consisting in raising them to a predetermined high temperature by conduction from heated bodies maintained at the desired temperature, and then chilling them.

2. The method of hardening thin steel blanks, consisting in raising them to the necessary high temperature by conduction from previously-heated solid bodies maintained at a substantially uniform temperature, and then chilling them by conduction from solid bodies of sufficient mass as to be substantially unaffected in temperature by contact with the blanks being treated.

3. The method of hardening thin steel blanks, consisting in raising them to a moderately-high temperature, subsequently raising them to a higher temperature by means of conduction from a previously-heated solid body, and then chilling them. 70

4. The method of hardening thin steel blanks, consisting in raising them to a moderately high temperature, subsequently raising them to a higher temperature by conduction from a previously-heated solid conductor, and then chilling them. 75

5. The method of hardening thin steel blanks, consisting in raising them to a moderately high temperature, subsequently confining them and raising them to a higher temperature when so confined, and chilling them. 80

6. The method of hardening thin steel blanks, consisting in raising them to a moderately high temperature, subsequently confining them and raising them to a higher temperature when so confined, and chilling them while confined under pressure. 85

7. The method of hardening razor blades 90 consisting in raising thin steel blanks to a moderately high temperature, subsequently confining them between suitable hot surfaces and raising them to a high temperature, subjecting them to the action of a blow 95 and of a chilling.

8. The method of hardening razor blades consisting in raising thin steel blanks to a moderately high temperature, subsequently confining them between suitable hot surfaces and raising them to a higher temperature and chilling. 100

9. The method of hardening razor blades consisting in raising thin steel blanks to a moderately high temperature, subsequently 105 confining them between suitable hot surfaces and raising them to a higher temperature and chilling between cold surfaces.

10. The method of hardening thin steel blanks consisting in heating them by conduction from another previously heated solid body maintained at a substantially uniform temperature, and chilling them. 110

11. The method of hardening thin steel blanks, consisting in heating and chilling 115 them by conduction from solid metallic bodies each of which is maintained at a substantially uniform temperature necessary to effect the heating and chilling operations. 120

12. The method of hardening thin steel blanks, consisting in heating them by conduction from previously heated solid bodies maintained at a substantially-uniform temperature, and then chilling them by contact with metal bodies maintained at the necessary low temperature. 125

13. The method of hardening thin steel blanks, consisting in raising them to the necessary high temperature by conduction 130

from and confining them by previously-heated solid bodies maintained at a substantially-uniform high temperature, and then chilling them by confinement by and contact with solid bodies maintained at the necessary low temperature.

14. The method of hardening razor blades consisting in raising thin steel blanks to a moderately high temperature, subsequently 10 confining them between suitable hot surfaces and raising them to a high temperature, subjecting them to the action of a blow and then chilling.

15. The method of uniformly hardening a 15 series of thin steel blanks consisting in raising them to the necessary high temperature by conduction from a heated body maintained at the desired temperature, and chilling them by contact with a cold body maintained at 20 a substantially uniform temperature.

16. The method of hardening a series of thin steel blanks uniformly, consisting in raising them to the necessary high temperature by inclosing them between heated 25 bodies maintained at a substantially uniform high temperature, and chilling them between cool bodies maintained at a substantially constant low temperature.

17. The method of hardening a series of thin steel blanks uniformly, consisting in 30 raising them to the necessary high temperature by inclosing them between heated bodies maintained at a substantially uniform high temperature, and chilling them by delivering them upon a cold metal block 35 and striking them with another cold block, both blocks being maintained at a substantially uniform low temperature.

18. The method of hardening a series of thin steel blanks, consisting in raising 40 them to the necessary high temperature by conduction from a heated body maintained at a substantially uniform high temperature, delivering them upon a solid body maintained at a uniformly low temperature, 45 and subjecting them while thus located to a blow from another solid body also maintained at a uniformly low temperature.

In testimony whereof, I have hereunto set my hand in the presence of two subscribing 50 witnesses.

WILLIAM E. NICKERSON.

Witnesses:

E. D. CHADWICK,  
OLIVER MITCHELL.